

H. P. BROWN,  
METHOD OF PRODUCING RAILWAY RAILS.  
APPLICATION FILED FEB. 4, 1911.

1,127,177.

Patented Feb. 2, 1915.

2 SHEETS—SHEET 1.



Fig. 1.



Fig. 2.



Witnesses:

Harry J. Bleischer  
J. George Barnes

Inventor: { *Harold P. Brown*  
*by his attorney*  
*Brown & Ward*

H. P. BROWN.

METHOD OF PRODUCING RAILWAY RAILS.

APPLICATION FILED FEB. 4, 1911.

1,127,177.

Patented Feb. 2, 1915.

2 SHEETS-SHEET 2.



Witnesses:

Harry J. Fleischer

J. George Barry

Inventor:

Harold P. Brown  
by his attorney

Mount & Ward

# UNITED STATES PATENT OFFICE.

HAROLD P. BROWN, OF MONTCLAIR, NEW JERSEY.

## METHOD OF PRODUCING RAILWAY-RAILS.

1,127,177.

Specification of Letters Patent.

Patented Feb. 2, 1915.

Application filed February 4, 1911. Serial No. 606,600.

To all whom it may concern:

Be it known that I, HAROLD P. BROWN, a citizen of the United States, and resident of Montclair, in the county of Essex and State of New Jersey, have invented a new and useful Improvement in Methods of Producing Railway-Rails, of which the following is a specification.

My invention relates to the method of producing railway rails, and more particularly to providing a railway rail with a wearing surface which shall have a greater resistance to wear than the body of the rail itself.

A practical embodiment of the invention is represented in the accompanying drawings in which,

Figure 1 represents a portion of a railway rail showing the method of depositing thereon a wearing surface by fusing a thin layer of pulverized manganese and melting it into the metal of the rail head or, by fusing a mixture of manganese oxid, aluminum and iron or steel filings and melting them on to or into the head of the rail to form a manganese steel wearing surface. Fig. 2 shows in transverse section a rail and means for forming a wearing surface thereon by melting pulverized manganese on the cleaned head of the rail and holding it in position by the steel clamp insulated from the rail itself. Fig. 3 illustrates the method of welding a bar or rod of manganese steel on the head of a rail and forming it in shape thereon. Fig. 4 illustrates the method of depositing manganese on the head of a rail by the use of a manganese electrode. Fig. 5 illustrates the method of rebuilding the low joints at the ends of the rails with manganese steel, and Figs. 6 and 7 show cross sections of rails provided with manganese steel wear-resisting layers on the top of the head and on the top and side of the head respectively.

Steel railway rails such as are in common use are subject to rapid deterioration and so great has the danger from wear and deterioration become that rails with from 12 to 18 per cent. of manganese have been put on the market for use on sharp curves or special work where the wear is abnormally great, but their use has been limited principally because of their high cost. This manganese steel is so tough that it cannot easily be worked with tools, files make no impression on it and holes cannot be drilled in it. On

the other hand, its stiffness is not so great as 55 that of carbon steel, and rails made of it have been found to sag between their supports. Its rate of wear, however, even on the most severe curves, is very small. For instance, on curves where a carbon steel rail 60 was practically worn out in from sixty to ninety days, a manganese steel rail has been in service for over three years with very slight wear.

The object of my present invention is to 65 retain the stiffness and moderate price of the steel rails such as are now used, while at the same time providing these rails with wearing surfaces of manganese steel or its equivalent, to materially lengthen their life 70 and increase their security.

My invention is further directed to a method of providing these rails with their wear-resisting surfaces without removing them from their position on the roadbed as 75 well as before they are laid in the track. To this end I have found that a strip of manganese steel, for example  $\frac{1}{4}$  to  $\frac{7}{16}$  inch thick and of the width of the worn rail can be rapidly and cheaply welded to the 80 head of the rail, by using preferably the electric arc with from 90 to 300 amperes and from 40 to 75 volts. The arc can be advanced along the rail, heating both the strip of manganese steel and the upper surface of the steel rail to a welding temperature. This method is illustrated in Fig. 3 of the drawings, where the rail is denoted by 1, the positive electrode, preferably of graphite, by 2, the holder for manipulating 85 the electrode by 3, a current regulator by 4, a source of electric energy by 5, and wires leading to the positive electrode and to the rail by 6 and 7. The strip of manganese steel is denoted by 8. The arc 34 from the 90 electrode 2 to the rail, which welds the strip to the rail, may be followed by a metal press 12 thrust downward by heavy pressure to compress the molten metal, and following this, a reciprocating hammer 9 100 to give a smooth wearing surface and to round the edge of the renewed rail on the gage line. Following this, a rapidly revolving wheel 10 may be pressed against the surface with comparatively light pressure to complete the surfacing and give a curve to the edge to fit the flange of the car 105 wheels. The surface may be finished by

grinding with the emery wheel 11. The strip 8 may be held in position by a suitable clamp 36

The metal of the thin strip or rod should preferably contain between 11 and 12 per cent. of manganese to make an alloy of the greatest resistance to wear. This alloy is tough but is not hard. It breaks with great difficulty. Its surface will withstand a great amount of mechanical service without parting with much of its material.

Instead of welding a rod or strip of manganese steel on to the surface of the rail, the manganese steel alloy may be formed and simultaneously welded on, as follows:

Referring to the structure shown in Fig. 1, the rail 1 has strips 13, 14, of magnesite or other highly refractory material clamped to its opposite sides and projecting somewhat above the upper surface of the head of the rail. Between these infusible strips may be placed on the head of the rail, the proper proportion of manganese oxid, for instance, what is commonly known as per-oxid of manganese, aluminum and iron or steel filings 35. There should be sufficient powdered aluminum, for instance one-fifth by weight of the manganese oxid, to rob the manganese oxid of its oxygen, releasing the manganese to unite with the steel. Steel filings to the amount of ten per cent. of the weight of the manganese can be used. These can then be melted by the electric arc 34 produced by an electric current through the wires 15, 16, from the source of electric energy indicated at 17, the wire 16 being electrically connected with the base of the rail and the wire 15 terminating in an electrode 18 in a support 19, which may be utilized to manipulate the electrode to fuse the constituent elements of the manganese steel alloy and at the same time weld them to the upper surface of the rail.

In the event a new rail is to be surfaced, the method may be carried out as indicated in Fig. 2, where the rail 1 is insulated from the clamp by means of suitable insulating material 20, and pulverized manganese, indicated at 21, may be held upon the head of the rail by the clamp and a heavy current of electricity may be passed from the source 22, through the wires 23, 24, one connected with the rail and the other with the clamp above the powdered manganese and the powdered manganese thereby carried into the surface of the rail by the action of the heat and the current to form a wear-resisting alloy. The temperature for this purpose should be from 500° to 800° F. The clamp may be insulated from the sides of the rail head by suitable insulating pieces 25, 26. Again, the manganese may be deposited in the surface of the rail directly from a manganese electrode 27, see Fig. 4, by means of the electric arc 34, forming

with the surface of the rail, manganese steel alloy. This is accomplished by moving the manganese electrode back and forth across the wearing surface of the rail, fusing the surface of the rail and at the same time depositing manganese from the electrode into the fused surface.

Low joints in rails may be built up as shown in Fig. 5, by first cutting away the ends of the rails on a slant, as indicated by the lines 28, 29, Fig. 5, then applying wedge-shaped pieces 30, 31, of manganese steel and welding these to the rail by the electric arc, as hereinbefore described.

When the constituents of the alloy are applied in the proper proportions and simultaneously melted together and welded into the rail, the aluminum seizes the oxygen from the manganese oxid, forming a slag which rises to the surface and releases pure metallic manganese which will unite at once with the melted steel. After cooling, the slag which is an abrasive, can be easily removed since it is quite brittle, but any portion of it extending into the surface of the rail will add to the friction coefficient and will also aid in resisting wear. Again, the friction coefficient can be increased by introducing carborundum in a powder or paste at the time the manganese steel is fused and welded on to the surface of the rail, or iron or steel filings mixed with an abrasive like carborundum in powdered form can be melted into the surface of the rail by the electric arc, thereby materially increasing the wear-resisting quality of the surface.

Where the track is straight, the wear-resisting surface may be applied to the top of the head of the rail only, as indicated in Fig. 6, where the wear-resisting laminum or surface is indicated by 32, and where the rails are laid on a curve the wear-resisting laminum or surface may be carried along the top and down the inner side of the head of the outer rail as indicated by 33, Fig. 7.

While I have indicated the electric arc and prefer to use the electric arc for performing the welding and fusing of the parts, other sources of heat might be employed with greater or lesser success, as, for instance, the oxy-acetylene blow pipe or the gasoline torch with compressed gas, or the welding can be accomplished by means of the welding apparatus using alternating current with a transformer and obtaining a welding current of great heating capacity from the secondary of the transformer, passing it through the metals to be welded. Again, although manganese steel is preferred as the wear-resisting surface, there are other alloys with wear-resisting properties greater than ordinary carbon steel. Among these would be vanadium steel, tungsten steel, chromium steel and nickel steel.

Nickel steel is, however, very slippery, especially so under certain weather conditions. Tungsten steel is somewhat brittle and vanadium steel has more elasticity than is required for this purpose and therefore so far as my experiments have thus far gone, manganese steel is preferred.

In carrying the method into practical effect on rails located in a track, the intense heat of the arc is localized on the upper surface of the rail and the process may be so rapidly completed that the temperature of the rail at the base will not injure the wooden tie.

15 In present practice a rail weighing say 100 lbs. to the yard and 5 to 6 inches in height is now discarded and replaced when but  $\frac{1}{8}$  of an inch has been worn from its head. By my process the wearing surface 20 of this rail can be restored without removing it from the track and the renewed rail will

then withstand a longer period of service than at first on account of the wear-resisting nature of the manganese steel head.

What I claim is:

1. The method of increasing the life of railway rails, consisting in simultaneously producing a steel alloy of greater wear-resisting properties than carbon steel and welding the same to the rail.

2. The method of increasing the life of railway rails, consisting in simultaneously producing manganese steel and welding it to the surface of the rail.

In testimony, that I claim the foregoing 35 as my invention, I have signed my name in presence of two witnesses, this second day of February 1911.

HAROLD P. BROWN.

Witnesses:

F. GEORGE BARRY,  
HENRY C. THIEME.